

# UNITED STATES PATENT OFFICE.

WALTER F. BURDEN, OF VICTORIA, BRITISH COLUMBIA, CANADA.

## CALCIMINE.

1,359,228.

Specification of Letters Patent. Patented Nov. 16, 1920.

No Drawing.

Application filed February 26, 1920. Serial No. 361,432.

To all whom it may concern:

Be it known that I, WALTER F. BURDEN, a subject of the King of Great Britain, and a resident of the city of Victoria, in the Province of British Columbia, Canada, have invented a certain new and useful Composition of Matter to be Used as Calcimine; of which the following is a specification.

The composition consists of the following ingredients, combined in the proportions stated for one ton of calcimine, viz:—

|                 |            |
|-----------------|------------|
| China clay      | 400 lbs.   |
| Ground whiting  | 1,419 lbs. |
| Cold water glue | 125 lbs.   |
| Lead acetate    | 30 lbs.    |
| Powdered alum   | 25 lbs.    |
| Oleate of lead  | 1 lb.      |
|                 | 2,000 lbs. |

These ingredients are to be thoroughly mixed together and the resulting composition used and applied as a calcimine in the well-known manner.

Calcimine consisting of the above ingredients may be prepared at less cost than similar compounds on account of the comparatively small proportion of glue used; it will take more water and therefore spread easier and cover more surface. A further advantage is that, as the effect of the lead acetate is to make the glue hard, the first coat of calcimine does not soften and mix with the second coat when being applied,

as occurs with other calcimine compounds, 35 also the respective coats do not perish and decay as in straight glue calcimine.

The oleate of lead may or may not be used, but if dispensed with an additional pound of whiting should be added to make 40 up the weight per ton.

What I claim as my invention is:

1. The herein described composition of matter comprising china clay, ground whiting, cold water glue, lead acetate, and powdered alum. 45

2. The herein described composition of matter consisting of china clay, ground whiting, cold water glue, lead acetate, powdered alum, and oleate of lead. 50

3. The herein described composition of matter comprising china clay four hundred pounds, ground whiting fourteen hundred and twenty pounds, cold water glue one hundred and twenty-five pounds, lead acetate thirty pounds, and powdered alum twenty-five pounds. 55

4. The herein described composition of matter, consisting of china clay four hundred pounds, ground whiting fourteen hundred and nineteen pounds, cold water glue one hundred and twenty-five pounds, lead acetate thirty pounds, powdered alum twenty-five pounds, and oleate of lead one pound. 60

Signed at Victoria, B. C., Canada, this Jan. 22, 1920.

WALTER F. BURDEN.